

# United States Patent Office

2,816,829

Patented Dec. 17, 1957

1

2,816,829

## NODULAR IRON MANUFACTURE

Harold N. Bogart, Detroit, Mich., assignor to Ford Motor Company, Dearborn, Mich., a corporation of Delaware

No Drawing. Application November 7, 1955  
Serial No. 545,531

5 Claims. (Cl. 75—130)

This invention is addressed to those interested in ferrous metallurgy and will be found to be of especial interest to the metallurgist engaged in the manufacture of nodular cast iron.

Nodular cast iron has attained great prominence in the ferrous metallurgy field in recent years and is characterized by an as-cast structure in which the graphitic carbon is in a round or nodular form as opposed to the graphitic flake usually associated with grey cast iron.

The manufacture of nodular cast iron usually involves the preparation of a low sulfur high carbon liquid grey cast iron composition to which is added usually in the ladle a ferro-alloy containing magnesium or cerium followed by an inoculation with ferro-silicon. This double treatment causes the precipitation of the graphitic carbon in the nodular form upon solidification and results in much higher physical properties than can be attained from conventional grey iron. By judicious manipulation of the silicon content the matrix may be made all pearlitic or all ferritic or any desired intermediate structure.

This invention is specifically aimed at a reduction in the overall cost of producing nodular iron by altering the inoculation procedure so that all or at least a portion of the ferro-silicon inoculant may be added in the molten form as opposed to the solid ferro-silicon which has been universally employed to date. In using solid ferro-silicon additions the art has found it necessary to employ ferro-silicon having a high silicon content to enable the addition of the requisite amount of silicon without unduly chilling the metal. When the silicon is added in the form of a molten iron silicon alloy, the silicon content of the alloy can be much lower inasmuch as no substantial amount of heat is abstracted from the metal by the addition. In fact, under some circumstances, the ferro-silicon may be heated sufficiently to add to the temperature of the base metal. The cost of producing iron silicon alloys, either molten or solid, goes up rapidly with the silicon content. Accordingly, it is much more economical to add a given amount of silicon as a low silicon content iron silicon alloy than as the higher grades of ferro-silicon.

As a specific example of the execution of this process a molten base iron was prepared in a standard three phase direct arc furnace. This alloy contained about 4 percent of carbon, .60 percent manganese, about 2 percent of silicon with minor amounts of phosphorus and a quite low sulfur content.

This furnace has been designated as "C" furnace in the data which follows. A second alloy was prepared in a Detroit rocking furnace (indirect arc furnace). This furnace was designated "B" furnace and was charged with 35 pounds of charcoal pig and 70 pounds of 16 percent silvery pig to give a bath having a silicon content of about 10 percent. From these two batches of molten metal eleven compositions were prepared as follows:

(1) Base iron in "C" furnace, carbide slag: 350# charcoal pig+1% Mn and .15% Cr.

2

(2) Alloy in "B" furnace: 35# charcoal pig, 70 lbs. silvery pig (16%) = 100% Si approx.

50# lots were made up by combining 1 and 2 in varying proportions as indicated, with and without a final solid inoculant. Test bars and fractures were cast.

Control: 50# from "C" furnace, added .55% solid FeSi, .15 Mg as MgCeFeSi; added .3% silicon (solid).

- 10 (a) 45# from "C" furnace, added .15% Mg as MgCeFeSi; added 5# from "B" furnace.  
(b) Added .2% solid FeSi to balance of (a).  
(c) 42# from "C" furnace, added .15% Mg as MgCeFeSi, added 8# from "B" furnace.  
(d) Added .2% solid FeSi to balance of (c).  
(e) 39# from "C" furnace, added .15% Mg as MgCeFeSi, added 11# from "B" furnace.  
(f) Added .2% solid FeSi to balance of (e).  
(g) 36# from "C" furnace, added .15% Mg as MgCeFeSi; added 14# from "B" furnace.  
(h) Added .2% solid FeSi to balance of (g).  
(i) 33# from "C" furnace, added .15% Mg as MgCeFeSi; added 17# from "B" furnace.  
(j) Added .2% solid FeSi to balance of (i).

25 Test bars were produced from each of these eleven compositions and these test bars were fractured and also polished and etched with the following results:

|         | Fractures                                                        | Microstructures                                                                               |
|---------|------------------------------------------------------------------|-----------------------------------------------------------------------------------------------|
| Control |                                                                  | 40-100% nodular (expl.), 5-10% Fe.<br>98% nodular, 2% ferritic.<br>98% nodular, 30% ferritic. |
| a.      |                                                                  | 95-98% nodular, 30-40% ferritic.                                                              |
| b.      |                                                                  | 98% nodular (expl.), 50% ferritic.                                                            |
| c.      | Fully nodular progressively finer grain with increasing silicon. | 98% nodular (expl.), 60-70% ferritic.                                                         |
| d.      |                                                                  | 50-90% nodular (expl.), 80% ferritic.                                                         |
| e.      |                                                                  | 95-98% nodular (expl.), 60% ferritic.                                                         |
| f.      |                                                                  | 95-98% nodular (expl.), 90% ferritic.                                                         |
| g.      |                                                                  | 98% nodular, 85-90% ferritic.                                                                 |
| h.      |                                                                  | 50-90% nodular (expl.), 90% ferritic.                                                         |
| i.      |                                                                  |                                                                                               |
| j.      |                                                                  |                                                                                               |

Each of these compositions were also fabricated into tensile test bars and tested with the following results:

|         | Physical properties |                  |                       |
|---------|---------------------|------------------|-----------------------|
|         | Yield strength      | Tensile strength | Percentage elongation |
| Control | 55,800              | 106,000          | 6                     |
| a.      | 59,000              | 86,000           | 4                     |
| b.      | 60,200              | 89,500           | 7                     |
| c.      | 62,000              | 87,000           | 6                     |
| d.      | 63,000              | 88,500           | 8                     |
| e.      | 69,400              | 93,500           | 6                     |
| f.      | 73,800              | 93,000           | 8                     |
| g.      | 76,000              | 92,000           | 2                     |
| h.      | 80,000              | 96,100           | 2                     |
| i.      | 86,700              | 89,500           | 0                     |
| j.      | 89,000              | 98,500           | 1                     |

|         | Reduction of area | Young's modulus |
|---------|-------------------|-----------------|
| Control | 6                 | 23.4            |
| a.      | 4                 | 23.4            |
| b.      | 7                 | 23.5            |
| c.      | 6                 | 23.5            |
| d.      | 9                 | 23.7            |
| e.      | 6                 | 23.8            |
| f.      | 8                 | 24.2            |
| g.      | 2                 | 24.2            |
| h.      | 2                 | 24.0            |
| i.      | 0                 | 23.2            |
| j.      | 1                 | 24.3            |

3  
The chemistry of these bars is as follows:

*Chemistry*

|         | O    | Mn  | Si   | P    | S    | Cr  | Mg   |
|---------|------|-----|------|------|------|-----|------|
| Control | 4.00 | .60 | 2.00 | .029 | .006 | —   | —    |
| a       | 3.93 | .89 | 3.29 | —    | —    | .24 | .030 |
| b       | 3.80 | .88 | 3.29 | —    | —    | .24 | .025 |
| c       | 3.82 | .88 | 3.58 | —    | —    | .24 | .027 |
| d       | 3.77 | .82 | 3.35 | —    | —    | .23 | .028 |
| e       | 3.69 | .83 | 4.03 | —    | —    | .25 | .034 |
| f       | 3.61 | .83 | 4.18 | —    | —    | .25 | .033 |
| g       | 3.36 | .85 | 4.43 | —    | —    | .25 | .028 |
| h       | 3.51 | .79 | 4.45 | —    | —    | .24 | .028 |
| i       | 3.44 | .79 | 4.96 | —    | —    | .25 | .033 |
| j       | 3.35 | .79 | 5.04 | —    | —    | .25 | .031 |

A study of the above data will demonstrate that it is readily possible to fabricate commercially acceptable and substantially completely nodular iron using molten ferro-silicon as the inoculant. The last several alloys are too high in silicon for most commercial usage and this high silicon is reflected in the low elongation and reduction in area in values. However, all of these specimens exhibit a Young's modulus of 23 or 24 million pounds per square inch which is very high for this class of material. All of these tests were made on unheat treated or as cast specimens.

While magnesium and cerium have been disclosed as the preferred initial inoculating agents, the invention is not so limited. Any of the divers inoculants disclosed in the nodular iron literature may be employed.

While a ten percent silicon content of the molten additive has been disclosed above, commercial considerations will usually dictate a somewhat lower silicon content, probably in the range of six percent of silicon. However, if weighing operations can be conducted accurately and the cost of higher grades of ferro-silicon is not a factor, any available ferro-silicon may be used. Circumstances favoring a high ratio of base metal to ferro-alloy is a high silicon content of the base metal, a high silicon ferro-silicon and a high silicon content in the cerium or magnesium containing additive. Under extreme conditions this ratio may be as high as twenty to one. Ordinary commercial production aimed at a three per cent silicon content in the final casting and employing a six percent silicon ferro-silicon calculates to slightly more than two parts of base metal to one part of ferro-silicon.

In the above description reference has been made to ferro alloys containing a nodularizing agent. These are usually preferable for economic reasons although other non-ferrous, nodularizing agents such as magnesium nickel or magnesium copper may be employed if special circumstances warrant.

I claim as my invention:

1. The process of producing nodular iron castings comprising preparing a molten alloy comprising iron, silicon and carbon of such composition that if cast without inoculation would solidify to yield ordinary flake graphite containing grey iron, adding to this molten alloy a solid ferro-alloy containing a nodularizing agent, and then

adding to the combination a molten ferro-alloy containing a substantial amount of silicon and a solid alloy containing a substantial amount of silicon whereby the entire molten mass is caused to solidify with the graphitic carbon in the nodular form.

2. The process of producing nodular iron castings comprising preparing a molten alloy comprising iron, silicon and carbon of such composition that if cast without inoculation would solidify to yield ordinary flake graphite containing grey iron, adding to this molten alloy a solid ferro-alloy containing a nodularizing agent selected from the group consisting of cerium and magnesium and alloys of cerium and magnesium adding to the combination a molten ferro-alloy containing a substantial amount of silicon and a solid alloy containing a substantial amount of silicon whereby the entire molten mass is caused to solidify with the graphitic carbon in the nodular form.

3. The process of producing nodular iron castings comprising preparing a molten alloy comprising iron, silicon and carbon of such composition that if cast without inoculation would solidify to yield ordinary flake graphite containing grey iron, adding to this molten alloy a solid ferro-alloy containing a nodularizing agent, and then adding to the combination approximately one ninth of its weight of a molten ferro-alloy containing a substantial amount of silicon and a solid alloy containing a substantial amount of silicon whereby the entire molten mass is caused to solidify with the graphitic carbon in the nodular form.

4. The process of producing nodular iron castings comprising preparing a molten alloy comprising iron, silicon and carbon of such composition that if cast without inoculation would solidify to yield ordinary flake graphite containing grey iron, adding to this molten alloy a ferro-alloy containing a nodularizing agent and a molten ferro-alloy containing a substantial amount of silicon and a solid alloy containing a substantial amount of silicon whereby the entire molten mass is caused to solidify with the graphitic carbon in the nodular form.

5. The process of producing nodular iron castings comprising preparing a molten alloy comprising iron, silicon and carbon of such composition that if cast without inoculation would solidify to yield ordinary flake graphite containing grey iron, adding to this molten alloy a solid nodularizing agent, and then adding to the combination a molten ferro-alloy containing a substantial amount of silicon and a solid alloy containing a substantial amount of silicon whereby the entire molten mass is caused to solidify with the graphitic carbon in the nodular form.

50  
55  
References Cited in the file of this patent

UNITED STATES PATENTS

|           |               |               |
|-----------|---------------|---------------|
| 342,869   | Hadfield      | June 1, 1886  |
| 1,061,363 | Hadfield      | May 13, 1913  |
| 2,485,760 | Millis et al. | Oct. 25, 1949 |
| 2,527,037 | Smalley       | Oct. 24, 1950 |